

## UNITED STATES PATENT OFFICE

2,126,823

## METHOD OF MAKING A STIFFENED FABRIC

George Schneider, Montclair, N. J., assignor to  
Celanese Corporation of America, a corpora-  
tion of Delaware

No Drawing. Application September 14, 1935,  
Serial No. 40,561

4 Claims. (Cl. 154—2)

This invention relates to the preparation of stiffened fabrics and also to wearing apparel and other articles formed in whole or in part of such stiffened fabrics.

5 This application is a continuation-in-part of my application S. No. 737,933 filed August 1, 1934.

An object of my invention is to prepare fabrics of any desired degree of increased stiffness and in a simple and expeditious manner. Another object of my invention is to prepare wearing apparel consisting of or containing such stiffened fabric. Other objects of my invention will appear from the following detailed description.

Articles of wearing apparel and similar articles are made by laminating two or more layers of fabric or sheet material, at least one of which contains cellulose acetate or other derivatives of cellulose, by causing the cellulose acetate or other derivative of cellulose to coalesce, thus effecting an adhesion between the various layers of fabric forming the article. The coalescence of the fabric containing cellulose acetate or other derivative of cellulose may be effected by subjecting the assembly to a liquid medium containing substances which cause the cellulose acetate or other derivative of cellulose to soften or melt at elevated temperatures. In the making of stiffened fabrics by causing cellulose acetate or other derivative of cellulose filaments to at least partially coalesce, there enter many considerations that are of great importance from the point of view of manipulative steps, of coalescing agents that may be employed by manufacturers who would ordinarily engage in such work, and also from the point of view of the properties of the final product. Thus, the use of volatile liquids that are active solvents for cellulose acetate, for instance, at ordinary room temperatures, present several difficulties, such as rather high costs, disagreeable and often noxious odor and inability to control the degree of coalescence and consequent stiffening to the desired extent, or the areas where stiffening occurs.

I have found that by using liquids that are not active solvents for cellulose acetate at ordinary temperatures but which attack the same at elevated temperatures, as an aid to cause coalescence upon the application of heat and pressure, many advantageous results are attained. Since these liquids are not active solvents at ordinary temperatures, the degree of coalescence of the filaments may be controlled to any extent from slight closing of the interstices of the fabric to complete closing thereof, whereby the stiffness, impermeability and other properties of the ma-

terial may be controlled. Moreover, since coalescence takes place only upon application of heat and pressure, by applying heat and pressure only locally, ordinary or other special effects may be produced. Further, since coalescence takes place only upon application of heat and pressure, the handling of the article prior to coalescence is facilitated as the layers of the article during assembly and up to the time of application of heat are free from tackiness, sogginess and limpness. 5

The products formed by my invention may be used for any purpose where a stiffened and/or relatively impermeable fabric is desired. An important application of such products is wearing apparel which may be formed in whole or in part of fabrics or assembly of fabrics made or prepared in accordance with this invention. Thus, collars or cuffs may be formed entirely of the product of this invention. Alternatively, shirts may be made wherein the attached collars, neckbands, cuffs, fronts or bosoms are made of such products. Hats or parts of hats may likewise be formed of such material, as may also be the inner or sweat bands of hats, visors for caps, inner linings for cravats, stiffening material used in the inner portions of garments, such as coats, to help retain the shape thereof, etc. The fabrics of this invention may be used for a variety of other purposes, and indeed may be used for any industrial or technical purpose where fabric of increased stiffness and/or impermeability is required. 10 15 20 25 30

An important advantage of this invention is that the fabric or assembly of fabrics employed as starting material may first be cut, sewn or otherwise shaped quite readily, since they have the properties of and may be handled as ordinary fabrics. After the desired articles, such as collars, cuffs, or other wearing apparel or parts thereof are formed, they may be treated with the liquid 35 that aids in effecting the coalescence of the cellulose acetate fabric after exposure to elevated temperatures and then subjected to heat and pressure to impart the desired stiffness, adhesion of the various layers, and/or impermeability. 40 45 In this manner, the sewing of stiff or impermeable material is avoided.

Products of this invention have any desired degree of stiffness, which is relatively permanent, so that they may be subjected to repeated laundering without substantially losing their stiffness. In this manner, the use of starch or other extraneous stiffening materials during laundering may be avoided. 50

This invention may be carried out in a large 55

number of ways, particularly as to the nature of the fabric or number of fabrics employed, provided that cellulose acetate in any form, such as powder, film, yarns or filaments are present in the fabric if a single fabric is used, or in or near at least one of the fabrics if a plurality of fabrics are used.

If the cellulose acetate is present in the form of yarns or filaments, then there should be present in the product treated at least one layer of fabric, which either consists wholly of cellulose acetate yarn, or which is a mixed fabric containing yarn of cellulose acetate either in the warp or in the weft or both, in any desired degree of alternation, with yarns of other non-thermoplastic fibres such as cotton, regenerated cellulose, linen, wool or natural silk. This alternation may be, for instance, 1, 2, 3 or more cellulose acetate yarns with 1, 2, 3 or more yarns of cotton or other non-thermoplastic fibres. For convenience, the warp may be made with such alternation of cellulose acetate yarn and yarn of other fibres, while the weft may consist wholly of such cellulose acetate yarn or wholly of yarn of other fibres. However, the weft may consist of an alternation of such cellulose acetate yarns and non-thermoplastic yarns of other fibres, in which case, if the fabric is made in ordinary looms, the alternations will be preferably in two's or multiples of two's. If desired a fabric may be used in which either the warp or the weft consists wholly of cellulose acetate yarn while the other component consists of non-thermoplastic yarn.

Instead of employing a woven fabric, a knitted or netted fabric may be employed. Also a fabric containing mixed yarn containing both filaments of cellulose acetate and fibres of cotton or other non-thermoplastic material may be employed.

Only a single layer of fabric consisting wholly of cellulose acetate yarn or a single layer of any of the fabrics above described containing both cellulose acetate yarn or filaments and non-thermoplastic fibres may be treated by this invention, whereby relatively thin fabric having the desired degree of stiffness or impermeability throughout or only locally may be produced. Alternatively, 2, 3, 4 or more of such fabrics may be treated with the liquid that causes stiffening at elevated temperatures and heat and pressure applied to the whole surface to form a composite fabric that is united throughout or only in local areas, by application of heat and pressure only at the desired local areas.

In another, and in some cases preferred, method of carrying out the invention, one or more fabrics consisting wholly of non-thermoplastic yarns, such as cotton, linen, reconstituted cellulose, wool or silk, is assembled with one or more fabrics consisting wholly of cellulose acetate yarn or of a mixture of cellulose acetate yarn and filaments and yarn of non-thermoplastic fibres, as above described, may be treated by this invention, whereby a composite fabric made up of a plurality of layers may be made. If a product is to be produced wherein all the layers thereof are united, it is of importance where two or more layers of fabric consisting wholly of non-thermoplastic material is used, that at least one layer of fabric consisting of or containing cellulose acetate yarn be interposed between such layers of fabric.

In another form of my invention I may employ, as the intermediate layers of the assembly, or as the sheet material which is to be coalesced to bind the other sheets together, a fabric consisting wholly of non-thermoplastic yarns and

filaments which has been coated with cellulose acetate. This coating of cellulose acetate may be applied to the non-thermoplastic material by applying the same thereto in the form of a powder or as a slurry in a liquid carrier. The coating of cellulose acetate may also be applied to the non-thermoplastic fabric from a volatile solution of the cellulose acetate, which volatile solvent is permitted to evaporate prior to laminating the fabrics.

If desired, either the yarns or powder coating that contains cellulose acetate also may contain a white or colored pigment. For instance, titanium oxide, antimony oxide, lead oxide or carbonate, iron oxide, etc., may be added to the cellulose acetate. When white pigments are employed with the cellulose acetate, the product is whiter in color and is not glazed or shiny in appearance.

As instances of the manner that the various fabrics may be assembled, the following are given. In the case of collars, cuffs, etc., where an exterior of cotton or linen is desired, a layer of fabric consisting wholly of or containing cellulose acetate yarn, as above described, may be interposed between two layers of fabric consisting of cotton, linen or other non-thermoplastic fibres. An assembly that is also useful for such purposes comprises three layers of fabric consisting wholly of such non-thermoplastic yarns, with a layer of fabric consisting of or containing cellulose acetate yarn between each of such fabrics.

Where a product is desired having an exterior of fabric made of or containing cellulose acetate, this may be done by interposing a layer of fabric consisting wholly of non-thermoplastic fibres between two layers of fabric consisting of or containing cellulose acetate filaments, or by forming an assembly of three layers of fabric containing or consisting of cellulose acetate yarn with a layer of fabric consisting of non-thermoplastic fibres interposed therebetween. In this case the fabric of non-thermoplastic material may be of the desired construction to impart to the final product such properties as may be required due to its fabric structure.

These arrangements are given only by way of example, it being obvious that other arrangements with a less or greater number of layers of fabric may be employed to obtain any desired effects.

When an assembly of two or more fabrics is used, particularly in connection with wearing apparel or parts thereof, such as collars, cuffs, shirt bosoms, mats, etc., it is advantageous to cut and sew them together to the desired form before causing coalescence of the cellulose acetate filaments, since it is much more convenient to manipulate them before the desired stiffness and/or impermeability is imparted thereto.

The fabric or assembly of fabrics is, in accordance with this invention, treated with a liquid that acts on the cellulose acetate at elevated temperatures so as to cause the same to stiffen, but which is preferably not an active solvent at ordinary temperatures. For this purpose, it is preferable to compound a liquid by mixing together an alcoholic material having a relatively low boiling point which alcoholic material is a solvent for the cellulose acetate at elevated temperatures, and a plasticizer for the cellulose acetate. To the mixture of plasticizer and alcohol may be added water as desired. The plasticizer may or may not be soluble in the alcohol or alcohol/water mixture. The plasticizer may

be dissolved in the low boiling alcohol or be added thereto as a suspension. Small amounts of active solvents, for instance, acetone, may be added to the liquid.

5 As the alcohol constituent in the liquid that acts on the cellulose acetate at elevated temperatures, I prefer to use methyl alcohol, ethyl alcohol, isopropyl alcohol and the like. Mixtures of these alcohols may be employed or mixtures of 10 one or more of these alcohols with water may be used as one component of the medium that acts on the cellulose acetate at elevated temperatures. The percentage of alcohol in the liquid may vary within wide limits, however, it is preferable to 15 employ more than 50% alcohol.

Aqueous solutions of ethyl, methyl or isopropyl alcohol of 55 to 90%, particularly of about 80%, concentration are very useful for this purpose. An aqueous solution of the mono methyl ether 20 of ethylene glycol containing say about 20% of water may be substituted for all or a part of the alcohol employed in forming the liquid having effect on cellulose acetate at elevated temperatures.

25 The plasticizer employed admixed or dissolved in the alcohol or alcohol and water may be any suitable one for the particular cellulose derivative or mixture of cellulose derivatives employed in the intermediate layers of the fabric, which 30 intermediate layers are to be coalesced for the purpose of uniting the assembly. The plasticizers may be any of the high boiling solvents or softening agents as, for example, the aryl sulphonamides such as para ethyl toloul sulphonamide, the alkyl phthalates such as dimethyl phthalate, the dialkyl tartrates such as dibutyl tartrate, the alkoxy esters of polybasic organic acids such as diethoxy ethyl phthalate, the polybasic acid esters of the mono alkyl ethers of polyhydric alcohols such as diethylene glycol ethyl ether ester of phthalic acid, the alkyl esters of phosphoric acid such as triethylglycol phosphate, the aryl esters of phosphoric acid such as tricresyl phosphate, the mixed alkyl and aryl phosphates such as ethylglycol dicresyl phosphate, and camphor. Other high boiling plasticizers such as triacetin, 45 diacetin, etc., may be employed. The expression "high boiling" as employed herein is intended to mean boiling above 200° C.

50 The liquid employed as an aid in coalescing the cellulose acetate fabric may be applied to the fabric or assembly of fabrics in any suitable manner, such as by dipping, spraying, padding or brushing. A convenient manner of wetting the fabric or assembly is by padding the same with the liquid. After an assembly of two or more fabrics is treated, both sides of the assembly should be wetted with the liquid, as it is desirable that all of the layers of the fabric present be 55 wetted therewith when heat and pressure is applied.

The so-wetted fabric or assembly of fabrics is subjected to heat and pressure. This may be done by any suitable device, for instance, by hot ironing or by passing between pressure rolls, one or both of which are heated, or between a heated roller and a heated or cold plate or surface, or between a heated pressing iron or plate and a cold board or surface. The heating device 60 may be heated to the desired temperatures, for instance, 100 to 180° C. or more, and the pressure applied may be any desired pressure, for instance, from 10 to 600 pounds per square inch.

If heated devices that have desired designs, 75 such as stripes, dots, rectangles or other geo-

metric figures, and floral or other designs, embossed thereon are employed, novel effects are obtained. Since the alcohol and like liquids are not solvents for the cellulose acetate at ordinary temperatures, only those portions that come in 5 contact with the embossed portions of the heated device become stiffened and/or united, while the other portions retain the properties of the original fabrics. This local application of heat and pressure may be done by manually operated 10 means if desired.

If collars or cuffs or bosoms or other articles which are to be sewn onto shirts or other articles of apparel are to be formed, it is advantageous to cut the assembly of fabrics to the desired shape 15 or form and sew it to the shirt or other article prior to the application of the aqueous alcohol and the heat and pressure so that the assembly is stiffened by wetting with the aqueous alcohol and application of heat and pressure only after 20 the shirt or other article is completed.

The fabrics and articles obtained by this invention may be made more or less stiff as desired by controlling the amount of cellulose acetate yarns or filaments in the assembly of fabrics 25 being treated; the more cellulose present, the stiffer the resultant products. The fabrics or other articles may be rendered softer by the incorporation of plasticizers, such as diethyl phthalate, dimethyl phthalate, dibutyl tartrate, 30 etc., in the aqueous alcohol or onto or in the fabrics containing the cellulose acetate filaments or yarns.

In order further to illustrate my invention without being limited thereto, the following examples of liquids suitable to effect coalescence of 35 the cellulose acetate are given:—

*Example 1*

|                    | Parts by volume |    |
|--------------------|-----------------|----|
| Isopropyl alcohol  | 75              | 40 |
| Water              | 15              |    |
| Dimethyl phthalate | 10              |    |

*Example 2*

|                    |    |    |
|--------------------|----|----|
| Ethyl alcohol      | 72 | 45 |
| Water              | 18 |    |
| Dimethyl phthalate | 10 |    |

*Example 3*

|                                      |    |    |
|--------------------------------------|----|----|
| Ethyl alcohol                        | 72 |    |
| Water                                | 18 | 50 |
| Mono methyl ether of ethylene glycol | 10 |    |

For making fabrics to be used for making any desired article, there is employed an assembly of two layers of cotton or linen fabric with an interposed layer of fabric consisting wholly of acetone-soluble cellulose acetate filaments or a fabric containing both cellulose acetate yarn and cotton yarn in any of the desired constructions as has been described. This assembly is then wetted on both sides with any of the liquids described above. Thereupon the assembly is pressed with a hot iron or calender to cause the cellulose acetate filaments to coalesce to form a stiffening material in which the fabrics are 55 united. By controlling the degree of heat and pressure and/or selection of the types of fabrics employed, the degree of heat and pressure and/or selection of the types of fabrics employed, the degree of stiffness may be controlled. Generally 60 a semi-stiff fabric is formed, which retains its stiffness after repeated laundering so that the use of starch or like material is not required.

While this invention has been described particularly in connection with yarns or filaments of 75

cellulose acetate, such cellulose acetate yarns or filaments may be replaced in whole or in part by yarns or filaments of other esters of cellulose such as cellulose formate, cellulose propionate, cellulose butyrate, etc., or yarns or filaments of ethers of cellulose such as methyl cellulose, ethyl cellulose and benzyl cellulose, etc., in which case suitable liquids having the required properties for aiding coalescence under heat and pressure 10 will be selected.

It is to be understood that the foregoing detailed description is merely given by way of illustration and that many variations may be made therein without departing from the spirit 15 of my invention.

Having described my invention, what I desire to secure by Letters Patent is:

1. The method of imparting stiffness or other properties to collars, cuffs and like parts of wearing apparel consisting of layers of textile fabric, 20 one of which contains an organic derivative of cellulose, which comprises applying heat and pressure thereto at least locally in the presence of a liquid containing a substantial amount of water, an alcohol and a plasticizer selected from the group consisting of triacetin, diethyl phthalate, 25 dimethyl phthalate, dimethyl phthalate and dibutyl tartrate.

2. The method of imparting stiffness or other properties to collars, cuffs and like parts of wearing apparel consisting of layers of textile fabric, one of which contains cellulose acetate, which comprises applying heat and pressure thereto 5 at least locally in the presence of a liquid containing a substantial amount of water, an alcohol and a plasticizer selected from the group consisting of triacetin, diethyl phthalate, dimethyl phthalate and dibutyl tartrate. 10

3. The method of imparting stiffness or other properties to collars, cuffs and like parts of wearing apparel consisting of layers of textile fabric, one of which contains an organic derivative of cellulose, which comprises applying heat 15 and pressure thereto at least locally in the presence of a liquid containing an alcohol, from 15 to 18% of water and 10% of dimethyl phthalate.

4. The method of imparting stiffness or other properties to collars, cuffs and like parts of wearing apparel consisting of layers of textile fabric, one of which contains cellulose acetate, which comprises applying heat and pressure thereto at least locally in the presence of a liquid containing an alcohol, from 15 to 18% of water and 25 10% of dimethyl phthalate.

GEORGE SCHNEIDER.